# EUROPEAN PATENT APPLICATION

(11) **EP 1 679 725 A1**
(43) Date of publication of application: **12.07.2006**
(21) Application number: 04793091.2
(22) Date of filing: 28.10.2004
(51) Int. Cl.: H01F 1/26, H01F 1/33, H01F 41/02, B22F 3/00

(54) **METHOD FOR PRODUCING COMPOSITE SOFT MAGNETIC MATERIAL HAVING HIGH STRENGTH AND HIGH SPECIFIC RESISTANCE**

(30) Priority: 30.10.2003 JP 2003370335
(71) Applicant: Mitsubishi Materials PMG Corporation, Niigata-shi, Niigata 9508064 (JP)
(72) Inventor: MIYAHARA, Masahisa, c/o Niigata Plant, Niigata-shi, Niigata 950-8640 (JP); MORIMOTO, Koichiro, c/o Niigata Plant, Niigata-shi, Niigata 950-8640 (JP)
(74) Representative: Wiedemann, Peter
(86) International application number: PCT/JP2004/015983
(87) International publication number: WO 2005/043559

(57) **Abstract**

Provided is a composite soft magnetic material having high strength and high specific resistance. There is provided a method of producing a composite soft magnetic material having high strength and high specific resistance, including: heating mixture powder having a composition containing 0.05-1 wt% of polyimide resin powder having an average particle diameter of 1 to 100 µm, 0.002-0.1 wt% of fine amide-based wax powder having an average particle diameter of 1 to 20 µm, and the balance composed of insulating film-coated soft magnetic powder obtained by forming an insulating film on the surface of soft magnetic powder, at a temperature of 60 to 110 °C; filling the heated mixture powder in a mold which is heated at a temperature of 100 to 150 °C; compacting the heated mixture powder at a molding pressure of 700 to 1200 MPa to obtain a compact; and curing the obtained compact at a temperature of 225 to 300 °C.

## Description

### Technical Field

The present invention relates to a method of producing a composite soft magnetic material having high strength and high specific resistance and a composite soft magnetic material having high strength and high specific resistance, which is produced by the method. The method of producing the complex soft magnetic material is used for producing an injector part, an ignition part, an electronic valve core, and a motor core.

### Background Art

In general, as soft magnetic powder, there is known iron power, Fe-Si iron-based soft magnetic alloy powder, Fe-Al iron-based soft magnetic alloy powder, Fe-Si-Al iron-based soft magnetic alloy powder, Fe-Cr iron-based soft magnetic alloy powder, Ni-based soft magnetic alloy powder, or Fe-Co soft magnetic alloy powder. The iron powder includes pure iron powder, the Fe-Si iron-based soft magnetic alloy powder includes Fe-Si iron-based soft magnetic alloy powder containing 0.1-10wt% of Si and the balance composed of Fe and necessary impurities (for example, ferrosilicon powder containing 1-12 % of Si and the balance composed of Fe and necessary impurities, more particularly, Fe-3%Si powder), the Fe-Al iron-based soft magnetic alloy powder includes Fe-Al iron-based soft magnetic alloy powder containing 0.05-10 of Al and the balance composed of Fe and necessary impurities (for example, Alperm powder having a composition of Fe-15%Al), the Fe-Si-Al iron-based soft magnetic alloy powder includes Fe-Si-Al iron-based soft magnetic alloy powder containing 0.1-10 wt% of Si, 0.05-10 of Al and the balance composed of Fe and necessary impurities (for example, Sendust powder having a composition of Fe-9%Si-5%Al), the Fe-Cr iron-based soft magnetic alloy powder includes Fe-Cr iron-based soft magnetic alloy powder containing 1-20 % of Cr, if necessary, one or two of 5 % or less of Al and 5% or less of Si, and the balance composed of Fe and necessary impurities, the Ni-based soft magnetic alloy powder includes Ni-based soft magnetic alloy powder containing 35~85% of Ni, if necessary, one or two of 5% or less of Mo, 5% or less of Cu, 2% or less of Cr, and 0.5% or less of Mn, and the balance composed of Fe necessary impurities (for example, Fe-79%Ni powder), and the Fe-Co soft magnetic alloy powder includes Fe-Co iron-based alloy powder 10-60 % of Co, if necessary, 0.1-3% of V, and the balance composed of Fe and necessary impurities. (% means wt% for above)

An insulating film is formed on such soft magnetic powder to produce insulating film-coated soft magnetic powder and the insulating film-coated soft magnetic powder is hardened with resin to produce a composite soft magnetic material. As the insulating film-coated soft magnetic powder, there are known oxide film-coated soft magnetic powder formed by performing high-temperature oxidation treatment on the soft magnetic powder to form an oxide film on the surface thereof, phosphate film-coated soft magnetic powder formed by performing phosphate treatment on the soft magnetic material to form a phosphate film on the surface thereof, and hydroxylation film-coated soft magnetic powder formed by performing stream treatment on the soft magnetic powder to form an insulating hydroxylation film on the surface thereof. Among these insulating film-coated soft magnetic powders, phosphate film-coated soft magnetic powder obtained by forming a phosphate film on the surface of pure iron powder is generally used.

As a method of hardening the insulating film-coated soft magnetic powder with the resin to produce a composite soft magnetic material, there is a method of filling mixture resin powder obtained by mixing 0.2-10 wt% of polyphenylenesulfide resin powder which is a thermoplastic compound having a particle diameter of 1 to 100 µm and 0.05-1 wt% of stearic acid powder having a particle diameter of 1 to 100 µm to the insulating film-coated soft magnetic powder in a mold which is heated to a temperature of 50 to 90 °C, compression-molding the mixture resin powder to produce a compact, curing the obtained compact at a temperature of 200 to 270 °C in a nitrogen atmosphere to remove the stearic acid, and heating the compact at a temperature of 285 to 310 °C in a nitrogen atmosphere (see Patent Document 1).

The method of hardening the insulating film-coated soft magnetic powder with the resin to produce the composite soft magnetic material can provide an excellent composite soft magnetic material, because the polyphenylenesulfide resin has a high melting point and excellent heat resistance and has good heat resistance and insulation property even under a high temperature area. However, this method has inferior moldability, because the polyphenylenesulfide resin powder has a melting point of at least 200 °C. To this end, there is suggested a method of adding 1-99% of polyamide resin powder to polyphenylenesulfide resin powder to produce mixture resin powder, compression-molding mixture powder obtained by adding the 0.1-3 wt% of mixture resin powder to insulating film-coated soft magnetic powder to produce a compact, and curing the obtained compact at a temperature of 250 to 450 °C in a nitrogen atmosphere to produce a composite soft magnetic material (see Patent Document 2).
Patent Document 1: PCT Japanese Translation Patent Publication No. 2001-504283
Japanese Unexamined Patent Application Publication No. 2003-183702

### Disclosure of the Invention

### Problems to be Solved by the Invention

However, the composite soft magnetic material produced using mixture powder obtained by adding insulating film-coated soft magnetic powder to mixture resin powder composed of polyphenylenesulfide resin powder and the stearic acid or mixture resin powder composed of polyphenylenesulfide resin powder and polyamide resin powder need be cured at as high temperature as possible, because sufficient transverse rupture strength cannot be obtained when the composite soft magnetic material is cured at a low temperature. However, when the composite soft magnetic material is cured at the high temperature in order to improve the transverse rupture strength, the specific resistance of the composite soft magnetic material is reduced.

### Means for Solving the Problems

Accordingly, the present inventors researched into a method of producing a composite soft magnetic material having high strength and high specific resistance and obtained the researched result that mixture powder having a composition containing 0.05-1 wt% of polyimide resin powder having an average particle diameter of 1 to 100 µm, 0.002-0.1 wt% of fine amide-based wax powder having an average particle diameter of 1 to 20 µm, and the balance composed of insulating film-coated soft magnetic powder obtained by forming an insulating film on the surface of soft magnetic powder has good moldability, and a composite soft magnetic material obtained by heating the mixture powder at a temperature of 60 to 110 °C, filling the heated mixture powder in a mold which is heated at a temperature of 100 to 150 °C, compacting the heated mixture powder at a molding pressure of 700 to 1200 MPa to obtain a compact, and curing the obtained compact at a temperature of 225 to 300 °C has higher strength and higher specific resistance, in comparison with the conventional composite soft magnetic material.

According to a first aspect of the present invention, there is provided a method of producing a composite soft magnetic material having high strength and high specific resistance, including: heating mixture powder having a composition containing 0.05-1 wt% of polyimide resin powder having an average particle diameter of 1 to 100 µm, 0.002-0.1 wt% of fine amide-based wax powder having an average particle diameter of 1 to 20 µm, and the balance composed of insulating film-coated soft magnetic powder obtained by forming an insulating film on the surface of soft magnetic powder, at a temperature of 60 to 110 °C; filling the heated mixture powder in a mold which is heated at a temperature of 100 to 150 °C; compacting the heated mixture powder at a molding pressure of 700 to 1200 MPa to obtain a compact; and curing the obtained compact at a temperature of 225 to 300 °C.

As the insulating film-coated soft magnetic powder obtained by forming the insulating film on the surface of the soft magnetic powder, phosphate film-coated pure iron powder obtained by forming a phosphate film on the surface of pure iron powder is generally used.
According to a second aspect of the present invention, there is provided a method of producing a composite soft magnetic material having high strength and high specific resistance, including: heating mixture powder having a composition containing 0.05-1 wt% of polyimide resin powder having an average particle diameter of 1 to 100 µm, 0.002-0.1 wt% of fine amide-based wax powder having an average particle diameter of 1 to 20 µm, and the balance composed of phosphate film-coated iron powder obtained by forming a phosphate film on the surface of pure iron powder, at a temperature of 60 to 110 °C; filling the heated mixture powder in a mold which is heated at a temperature of 100 to 150 °C; compacting the heated mixture powder at a molding pressure of 700 to 1200 MPa to obtain a compact; and curing the obtained compact at a temperature of 225 to 300 °C.

### Effect of the Invention

It is possible to produce a composite soft magnetic material having higher strength and higher specific resistance, in comparison with the conventional composite soft magnetic material.

As the polyimide resin powder contained in the mixture powder used for the method of producing the composite soft magnetic material according to the present invention, wholly aromatic polyimide resin powder, bismalade-based polyimide resin powder, or additive polyimide resin powder may be used and the average particle diameter thereof is preferably in a range of 1 to 100 µm (preferably 10 to 80 µm, and more preferably 10 to 50 µm). This is because it is difficult to produce polyimide resin powder having an average particle diameter of 1 µm or less and it is impossible to obtain sufficient strength and high specific resistance when the polyimide resin power having an average particle diameter of 100 µm or more is used. In addition, the amount of the polyimide resin powder contained in the mixture powder is preferably in a range of 0.05 to 1 wt% (more preferably 0.1 to 0.5 wt%). This is because sufficient specific resistance cannot be ensured when the amount of the polyimide resin powder contained in the mixture powder is less than 0.05 wt% and density, flux density, and magnetic permeability are reduced when the amount of the polyimide resin powder is greater than 1 wt%.
In addition to the polyimide resin powder, 0.002-0.1 wt% (preferably, 0.004-0.05 wt%) of fine amide-based wax powder having an average particle diameter of 1 to 20 µm (preferably, 1 to 10 µm) need be added to the mixture powder as lubricant. As the amide-based wax, simple substance of ethylenebisstearoidamide, ethylenebislauramide, or methylenebisstearoid or a mixture thereof may be used.
By adding the amide-based wax powder together with the polyimide resin powder, filling property of the polyimide resin is improved to suppress generation of a large triple point and crescent tear is prevented from occurring in the powder grain boundary due to extrusion of resin to the triple point to increase the density of the compact. However, when the amount of the amide-based wax powder contained in the mixture powder is less than 0.002 wt%, sufficient flow property cannot be ensured, and, when the amount of the amide-based wax powder contained in the mixture powder is greater than 0.1 wt%, the strength of the composite soft magnetic material is reduced.
Accordingly, the amount of the amide-based wax powder contained in the mixture powder is determined to 0.002 to 0.1 wt%. The average particle diameter of the amide-based wax powder added to the mixture powder is preferably in a range of 1 to 20 µm. This is because it is difficult to produce amide-based wax powder having an average particle diameter of 1 µm or less and the amount of the added material necessary for ensuring the flow property too increases and sufficient strength cannot be obtained when amide-based powder having an average particle diameter of 20 µm or more is used.
The mixture powder having such a composition is heated at a temperature 60 to 110 °C, and filled and compression-molded in a mold which is heated at a temperature of 100 to 150 °C. The reason why the mold is heated at the temperature of 100 to 150 °C is because, when colloidal lubricant agent is coated on a wall surface of the mold, moisture contained in lubricant agent is evaporated and the solid lubricant agent is attached to the wall surface of the mold. Accordingly, the heating temperature of the mold need be 100 °C or more, but need not be 150 °C or more. When the heating temperature of the mixture powder filled in the heated mold is less than 60 °C, the density of the compact does not increase, and, when the heating temperature of the mixture powder is greater than 110 °C, the flow property is reduced. Accordingly, the mixture powder filled in the mold is heated at the temperature of 60 to 110 °C.

The reason why the mixture powder filled in the mold is compression-molded at the pressure of 700 to 1200 MPa is because, when the compression molding pressure is less than 700 MPa, sufficient density cannot be obtained, and, when the compression molding pressure is greater than 1200 MPa, the specific resistance is reduced. The compact obtained by the compression molding is cured at a temperature of 225 to 300 °C for 30 to 60 minutes. By curing at the above-described temperature, a composite soft magnetic material having high strength and high specific resistance is obtained. In addition, by curing at the above-described temperature, distortion of the soft magnetic powder is removed and soft magnetic property is restored. The reason why the curing temperature is limited to 225 to 300 °C is because the resin is insufficiently hardened when the curing temperature is less than 225 °C and the strength and the specific resistance are reduced due to the decomposition of the resin when the curing temperature is greater than 300 °C.
According to the method of producing the composite soft magnetic material using the polyimide resin powder, it is possible to produce a composite soft magnetic material having higher strength and higher specific resistance, in comparison with the conventional composite soft magnetic material using the polyphenylenesulfide resin powder. This is because the polyphenylenesulfide resin has inferior distortion property and thus damages the insulating film of the insulating film-coated soft magnetic powder at the time of compression-molding at 700 to 1200 MPa to reduce the specific resistance. Meanwhile, when the ratio of the polyamide resin is large, the polyamide resin is too soft and thus crescent tear of the insulating film generated between the insulating film-coated soft magnetic powder and the insulating film-coated soft magnetic powder occurs, thereby reducing the specific resistance.

### Best Mode for Carrying out the Invention

### Embodiment

As a raw material, available phosphate film-coated iron powder having an average particle diameter of 80 µm, which is obtained by performing phosphate treatment on pure iron powder to form a phosphate film on the surface thereof, was prepared and additive polyimide resin powder and ethylenebisstearoidamide powder having average particle diameters shown in Table 1 were prepared. By adding and mixing the additive polyimide resin powder and the ethylenebisstearoidamide powder to the phosphate film-coated iron powder with a ratio shown in Table 1 in the atmosphere, mixture powders A to R of compositions shown in Table 1 were produced.

The mixture powders A to R were heated at temperatures shown in Tables 2 and 3. In addition, an aqueous solution including 1% of sodium benzoate and 1% of dipotassium hydrogen phosphate was sprayed and dried on a wall surface of a mold which is heated at temperatures shown in Tables 2 and 3, the heated mixture powders A to R were filled in the mold which is heated at the temperature shown in Tables 2 and 3 and compression-molded with pressures shown in Tables 2 and 3 to produce a compact, and the compact was heated for a time shown Tables 2 and 3 at the temperature shown in Table 2 and 3 in the atmosphere, thereby performing Present methods 1 to 12 and Comparative methods 1 to 13. Accordingly composite soft magnetic samples having a size of 5 mm x 10 mm x 60 mm were produced.
The transverse rupture strength, the density, the specific resistance, and the flux density of the composite soft magnetic samples were measured at a room temperature and the measured results were shown in Table 2 and 3.

### Conventional Example

Mixture powder obtained by adding and mixing 1 wt% of polyphenylenesulfide resin powder having an average particle diameter of 30 µm and 0.2 wt% of stearic acid powder having an average particle diameter of 30 µm to the insulating film-coated iron powder prepared in the embodiment was filled in a mold which is heated at a temperature of 70 °C and was compression-molded to produce a compact, the obtained compact was cured at a temperature of 230 °C in a nitrogen atmosphere to remove stearic acid, and the compact was heated at a temperature of 300 °C in a nitrogen atmosphere, thereby performing Conventional method 1.

In addition, mixture resin powder obtained by adding and mixing 50 wt% of polyphenylenesulfide resin powder having an average particle diameter of 18 µm and 50 wt% of polyamide resin powder to the phosphate film-coated iron powder prepared in the embodiment was produced, 1.5 wt% of mixture resin powder was mixed to phosphate film-coated iron powder to produce mixture powder, the obtained mixture powder was compression-molded to produce a compact, the obtained compact was cured at a temperature of 300 °C in a nitrogen atmosphere to produce a composite soft magnetic sample, thereby performing Conventional method 2. The transverse rupture strength, the density, the specific resistance, and the flux density of the composite soft magnetic samples obtained by Conventional methods 1 and 2 were measured at a room temperature and the measured results were shown in Table 2 and 3.

From the results shown in Table 2 and 3, it can be seen that the soft magnetic samples produced by Present methods 1 to 12 have more excellent soft magnetic property, compared with the soft magnetic samples produced by Conventional methods 1 to 2. In addition, the soft magnetic samples produced by Comparative methods 1 to 14 performed under a condition different from that of the present invention partially have inferior property.

## Claims

1. A method of producing a composite soft magnetic material having high strength and high specific resistance, comprising:
heating mixture powder having a composition containing 0.05-1 wt% of polyimide resin powder having an average particle diameter of 1 to 100 µm, 0.002-0.1 wt% of fine amide-based wax powder having an average particle diameter of 1 to 20 µm, and the balance composed of insulating film-coated soft magnetic powder obtained by forming an insulating film on the surface of soft magnetic powder, at a temperature of 60 to 110 °C;
filling the heated mixture powder in a mold which is heated at a temperature of 100 to 150 °C;
compression-molding the heated mixture powder at a molding pressure of 700 to 1200 MPa to obtain a compact; and
curing the obtained compact at a temperature of 225 to 300 °C.

2. The method of producing the composite soft magnetic material according to Claim 1, wherein the insulating film-coated soft magnetic powder is phosphate film-coated iron powder obtained by forming a phosphate film on the surface of pure iron powder.

3. A composite soft magnetic powder having high strength and high specific resistance, which is produced by the method according to Claim 1 or 2.
